

# UNITED STATES PATENT OFFICE.

EMIL POLLACSEK, OF NEW YORK, N. Y.

## PROCESS OF PREPARING AND REDUCING ORES.

No. 854,527.

Specification of Letters Patent.

Patented May 21, 1907.

Application filed October 18, 1904. Serial No. 229,042.

To all whom it may concern:

Be it known that I, EMIL POLLACSEK, a subject of the King of Hungary, and a resident of New York, borough of Manhattan, 5 county and State of New York, have invented certain new and useful Improvements in Processes of Preparing and Reducing Ores, of which the following is a full, clear, and exact description.

- 10 This invention relates to the preparation and reduction of ores, and has particular application to an improved process of preparing iron ores for smelting and conversion into iron and steel.
- 15 In carrying out my invention, I have especially in contemplation so treating the native ore and combining the same with certain agents and elements that a product is obtained, which, when subjected to the 20 smelting process in the blast furnace, will yield, at one operation, a superior grade of iron or steel, the character and quality of the resultant metal depending largely upon the quantity and nature of the components of 25 the mixture when first introduced into the furnace.

With the above recited objects and others of a similar nature in view, my invention consists in the improved process and the 30 product hereinafter claimed.

In the practice of my invention I employ either what is commonly termed "iron ore dust," or ore in its native rocky state, and in the latter case the ore is crushed until the 35 particles are reduced to granular form, and to the bulk I add, by mixing, certain basic agents such as lime, magnesia, or both, in sufficient quantities to unite with the silicates, phosphorus and phosphoric acid of the 40 ore, for the purpose of forming salts thereof and acting as the fluxing agent. The basic agents are preferably added in quantities in excess of the amounts theoretically required, in order to produce a rapid fusing and silicating and to retard the liberation of the phosphorus and similar agents, thus preventing 45 the latter combining with the metal in the form of protoxids and detrimentally affecting the smelting of the ores. It is also desir- 50 able to employ a surplus quantity of basic agents to act in conjunction with the small quantity of scrap iron, or iron shavings (used for the purpose hereinafter mentioned) to cause the formation of ferric hydrate— $Fe(OH)_3$ , when water is added to the compound, or mass, in the presence of air. Fi-

nally the basic agents should be present in the compound in such quantity as to effect a thorough reduction of the ore when in the blast furnace.

To the mixture of fine ore and the basic agent, I add a quantity of the above mentioned iron shavings or scrap iron, thus increasing the percentage of pure iron in the mass, and causing the formation of the ferric 60 hydrate (when water is present) which performs the function of a binding agent and causes the mass to harden without having recourse to pressure to accomplish such hardening. The term iron in this connection is 65 used in its ordinary sense, including steel and the various other forms of the metal. There is then added to the mass or composition a suitable reducing agent such as charcoal, coke, coal or wood dust, in such proportions 70 as may be found desirable for carbonating and for the reduction of oxids. The compound is then supplied with water in which a glue-like substance of organic nature has 75 been dissolved. While this glue-like sub- 80 stance may be of any desired character, I have found that for the purposes of my invention a material manufactured from wood pulp is preferable. This may be obtained in various ways; for instance, by subjecting the 85 wood pulp to pressure for the purpose of obtaining an extract which has the qualities of 90 adhesiveness and coherence, while at the same time it yields a relatively large percentage of carbon during the smelting opera- 95 tion. During the process of obtaining the extract there is added to the latter a suitable basic agent and acids for the purpose of neutralization.

The water containing the glue-like sub- 95 stance is added to the dry mixture of ore, basic agents, scrap iron, and reducing agent, in sufficient quantities to give to the mass a plastic consistency, the formation of the ferric hydrate occurring upon the addition of 100 the fluid. In such plastic state the composition is introduced into the blast furnace, the presence of the water preventing the mass drying too quickly and cracking or crumbling when exposed to the furnace heat. The glue- 105 like material disintegrates in the furnace and leaves a solid residue which forms an incrustation, thus further hardening the mass. In the highest smelting zone in the furnace this residue is freed of a relatively large quantity 110 of carbon which combines with the fused metal. The hardening of the mass should

take place slowly in order to prevent crumbling and disintegration through the escape of carbonic acid gas, and when the mass is exposed to a high temperature only a crust or shell should be formed. The surplus of basic agents serves as a fluxing agent during the final steps in the smelting process, and is drawn off as slag, along with the silicates from the metal.

10 10. What I claim is:

- 11 1. The herein described composition comprising an iron-containing body, a basic agent, a reducing agent and a binder containing a gluelike material.
- 12 2. The herein described composition consisting of iron ore, a basic agent, a reducing agent and water containing a gluelike material of organic origin.
- 13 3. A process of preparing ore for reduction,

which consists in mixing suitable proportions 20 of an iron-containing body, a basic agent, a reducing agent, and introducing to the mass a fluid containing a gluelike substance for the purpose of giving the mass a plastic consistency and combining together the components 25 of such mass.

4. A process of preparing ore for reduction and smelting which consists in mixing suitable proportions of an iron-containing body, a basic agent, a reducing agent, and a fluid 30 containing a gluelike material.

In testimony whereof I have signed my name to this specification in the presence of two subscribing witnesses.

EMIL POLLACSEK.

Witnesses:

G. LEVE,  
R. B. CAVANAGH.